

## UNITED STATES PATENT OFFICE

1,944,778

## METHOD OF PROTECTING LEAD AGAINST CORROSION

Henri Benit, Paris, France, assignor to Compagnie Generale D'Electricite, Paris, France

No Drawing. Application May 7, 1931, Serial No. 535,810, and in Germany May 7, 1930

REISSUED

3 Claims. (Cl. 173—266)

The corrosion of lead employed in the form of pipes or tubes and for sheathing electric cables exposed to the weather or buried in the soil or embeded in cement is well known.

5 In general, in order to prevent corrosion the lead is separated from the surrounding medium by covering it with a protective coating generally constituted by one or more layers of pitch or of tar, the coating being maintained and protected mechanically by a covering of jute or canvas. It is found in practice that such waterproof coatings do not always remain wholly impermeable, cracks are produced eventually in the layer of protective coating and infiltration 10 of moisture in the presence of air produces corrosion of the lead.

Moreover the substance used to form the protective coating should not itself contain products which are corrosive of lead or which become so 20 in the presence of other chemical agents contained in the soil; otherwise the lead will be destroyed eventually. It is thus necessary to employ a perfectly neutral protective coating which is much more costly in general than ordinary tars and the neutrality of which is often 25 difficult to verify.

The process forming the subject of the present invention avoids the above mentioned disadvantages. It consists in rendering the lead 30 unattackable by destructive agents by creating on its surface, chemically, a protective layer formed by a very stable lead salt which resists chemical changes. The lead salt thus produced will form a very thin layer protected mechanically by the usual covering which might now be 35 of ordinary tar or other inexpensive material which will not be chemically neutral. There will no longer be any liability of corrosion of the lead in case of cracking of the waterproof covering 40 even if corrosive products are present in this coating because the lead salt formed on the surface of the lead will prevent attack by the latter.

The lead salt which forms the protective 45 should be very stable and be easily and cheaply formed. Lead sulphide fulfils these conditions; it is insoluble in water and is unattackable or almost unattackable by acids and mineral and organic salts. It is formed easily from pure sulphur or from natural or artificial sulphide derivatives in contact with lead, the reaction being 50 very rapid with the aid of heat.

In accordance with the invention the protective layer is formed preferably by lead sulphide obtained simply by introducing an excess of sulphur 55 into the substance intended to serve as

the protective covering either in the form of pure sulphur which dissolves well in tar or pitch or in the form of natural or artificial sulphide derivatives.

For example, there may be applied to the lead 60 directly at a temperature a little above 100° C. a layer of ordinary tar mixed with pure sulphur in a proportion greater than 3%. Under these conditions there will be formed instantaneously on the lead a film-like coating of lead sulphide and 65 the reaction will cease of its own accord leaving an excess of sulphur in the tar.

The advantages of the process forming the subject of the invention are the following:

The superficial layer of lead sulphide protects 70 the lead against the action of phenols, cresols and other destructive agents contained in tar or in the protective covering employed, or which may be formed even in the presence of other chemical agents in the soil. The lead sulphide which 75 covers the surface of the lead protects the lead even in the case where the waterproof covering round the pipe or the lead sheathing is not completely impermeable to water. The lead sulphide even altered by oxidation continues to protect the lead by being converted into sulphate 80 which is equally insoluble or very slightly soluble in water.

The excess of sulphur contained in the layer 85 of tar continues to protect the lead by acting as a sulphidizing medium or as a sulphatizing medium after oxidation. This is important as it might happen that the first protective coating of sulphide would be impaired and the lead would be exposed. Under these conditions there would 90 still exist along the lead tube the sulphidizing and sulphatizing protective medium. On the other hand, the constant emission of sulphuric acid would oppose the dissolving action which 95 certain ammoniacal organic salts which are found in the soil (acetates, tartrates of ammonia etc.) exert on the sulphate of lead.

Where the protective covering for the lead consists of concrete or cement another form of the invention consists in incorporating in the cement 100 during the preparation of the mortar a small proportion of sodium sulphide. It will be understood, from what has been stated above, that the lead will thus be protected against attack of the most highly basic cements. This form of the invention is susceptible of very important applications because it permits of avoiding the corrosion of the lead in the very frequent instances where lead pipes pass through walls or masonry 105 or when electric cables covered with lead sheath- 110

ing are laid on shelves of cement in galleries or in sewers.

The process forming the subject of the present invention permits also of protecting the lead from electrolytic corrosion or at least of reducing greatly the destructive effects of electrolysis by retarding the speed of the reaction in the ratio of about 10:1 under the same conditions. In fact the oxygen liberated by electrolysis transforms the sulphide of lead into the sulphate which continues to protect the lead. In the presence of an excess of sulphur in the tar sulphuric acid will be formed which will assist to maintain the protective medium in contact with the lead in the sulphidizing and sulphatizing state.

Having now particularly described and ascertained the nature of my said invention and in what manner the same is to be performed, I declare that what I claim is:

20 1. In a method of preventing corrosion of the lead sheathing of electric cables wherein the lead sheathing is protected against mechanical deterioration by a layer of a suitable covering material not chemically neutral and not adapted to protect the lead against corrosion, incorporating sulphur to the said protective materials in such quantity that on contact of the lead with these materials a film of lead sulphide will be immediately formed thereon and there will remain 25 in the said protective materials an excess of sulphurating material constantly active to renew any worn portion of the said lead sulphide film, and so prevent the destructive effects of electrolytic phenomena on the lead.

35

80

85

90

2. In a method of preventing corrosion of the lead sheathing of electric cables wherein the lead sheathing is protected against mechanical deterioration by a layer of a suitable covering material not chemically neutral and not adapted to protect the lead against corrosion, incorporating to the said protective materials quantities of sulphur derivatives having a sulphurating action on lead such that on contact of the lead with these materials there will be immediately formed on the lead a film of lead sulphide and there will still remain in the said protective materials an excess of sulphurating material active to constantly renew any worn portion of the said lead sulphide film, and so prevent the destructive effects of electrolytic phenomena on the lead.

3. In a method of preventing corrosion of the lead sheathing of electric cables wherein the lead sheathing is protected against mechanical deterioration by a layer of a suitable covering material not chemically neutral and not adapted to protect the lead against corrosion, incorporating to the said protective materials a quantity of sodium sulphide such that on contact of the lead with these materials a film of lead sulphide will be immediately formed on the lead sheathing and there will still remain in the said protective materials an excess of sulphurating material constantly active to renew any worn portion of the said lead sulphide film, and so prevent the destructive effects of electrolytic phenomena on the lead.

HENRI BENIT.

95

40

100

105

45

110

50

115

55

120

60

125

65

130

70

135

75

140

145

150